

## UNITED STATES PATENT OFFICE

2,088,193

LUBRICANT AND METHOD OF PRODUCING  
SAMEWilliam L. Evers, Woodbury, N. J., assignor to  
Socony-Vacuum Oil Company, Incorporated,  
New York, N. Y., a corporation of New YorkNo Drawing. Application February 27, 1935,  
Serial No. 8,554

7 Claims. (Cl. 87—9)

This invention is concerned with lubricants for use as extreme pressure lubricants or, in general, for lubrication under conditions characterized by unusually high unit loading at point of application of lubricant, and it has specifically to do with ingredients and combinations of ingredients for use in the making of such oils, the manner of production of such ingredients, and the manufacture of the lubricants therefrom.

10 Extreme pressure lubricants must be capable of withstanding extremely high unit loading. Typical applications are the lubrication of free wheeling devices, certain forms of ball-bearing power transmission devices, certain forms of gear tooth characterized by high tooth pressure, metal cutting, and similar instances. Extreme pressure lubricants are usually compounded from oils of high viscosity and the oil plays some part in the lubrication, although the major portion of the effectiveness is because of the presence of a characterizing ingredient. Ingredients for lubricants of these types have been of various forms. This invention has to do specifically with novel ingredients of this nature and their method of manufacture, the invention contemplating the ingredient alone or in combination with other ingredients to form the active portion of lubricants for the above indicated use, and the complete lubricant.

20 It is an object of this invention to produce a novel and valuable base for such lubricants, to prepare such a base having good characteristics of stability, and to provide means for the preparation of such ingredients. A further object is the preparation of extreme pressure lubricants characterized by the presence of these ingredients alone or in combination with other ingredients. Further objects are the provision of methods of preparing lubricants and such other objects and advantages as may hereinafter appear.

30 The preparation of the novel ingredients for extreme pressure lubricants in accordance with this invention is effected by first interacting a mercaptide or mercaptides with one or more halo-45 gen-substituted fatty acids, or alkali metal salt, or salts thereof, or other metallic salts thereof which are soluble in the mercaptide reaction, followed by the preparation of a reaction product from such mercaptio substituted fatty acid and 50 stannic chloride. Chlor-substituted fatty acids

are preferred. The preferred range of fatty acids is from butyric to caprylic, inclusive. The first step of the process just mentioned produces a new composition of the general formula



5 where R is any alkyl or aryl radical. If a metal salt of the fatty acid is used, the reaction product will be of the general formula  $RS(CH_2)_xCOOM$ , where M is the metal. The M is displaced with H by acidifying the solution, as with hydrochloric or sulfuric acid. Then stannic chloride may be incorporated with the above resulting organic acid. The product of this second reaction has been found to exhibit novel and characteristic 10 ability for imparting load bearing capabilities to hydrocarbon lubricants, together with an unusual 15 stability and other desirable qualifications for such purpose.

20 As an example of the preparation of one of these novel ingredients, I may cite the following: Chloracetic acid ( $ClCH_2COOH$ ) may be converted to its sodium salt, for example, by dissolving in a caustic soda solution, and this sodium salt reacted with a sodium mercaptide or a mixture of sodium 25 mercaptides typified by the general formula  $RSNa$  where R indicates any alkyl or aryl radical. This reaction is capable of proceeding under its own heat of reaction, but I prefer to apply heat sufficient to maintain a temperature in the range 30 of 60 to 70° C. in order to obtain high yields. For maximum yield the fatty acid and mercaptide should be reacted in stoichiometric proportions, altho this is not essential to the purposes of this 35 invention. After completion of this first reaction, the reaction mixture is introduced into acidified water which takes out any salt, sodium or unreacted chloracetic acid, and also reacts with the sodium salt which is the first reaction product; the oily reaction product of the second 40 reaction separates as a top layer, is taken up with ether, and any unreacted mercaptan removed by distillation, leaving the desired second reaction product. The product obtained from the process at this stage of reaction is an oily substance, 45 which may be typified by the formula



This oily product I then incorporate with stannic chloride ( $SnCl_4$ ) in desired amount, say from 5% to 30%, for example about 10% by weight of 50

stannic chloride, not in such large amount as to separate out when the finished product is mixed into mineral lubricating oil at room temperature. This second reaction is also exothermic. I have found that it usually results at first in the formation of a white precipitate which subsequently dissolves. No evolution of hydrochloric acid gas is observed. The resultant compound is probably  $(RSCH_2COOH)_2SnCl_4$  [or, for any fatty acid the general formula will be  $(RS(CH_2)_xCOOH)_2SnCl_4$ ], in a solution of mercapto acid and/or an excess of stannic chloride. The formation of a precipitate and evolution of heat point to the formation of an addition compound. However, it is not certain that the final compound attained is of this type, and for purposes of definition, I choose to indicate my final product, which is the subject matter of this invention, as the reaction product of stannic chloride and a mercaptan containing organic acid. This compound, I have found to be capable of serving as a characterizing ingredient in extreme pressure lubricants to enable them to withstand high unit loading. In the formation of my preferred compound, I prefer to incorporate about 10% stannic chloride with the mercaptan-containing organic acid. The particular halide also may be iodine or bromine as well as chlorine, insofar as these other halides form substituted acids capable of performing reactions of this type. Mixed mercaptides and mixed metal salts of fatty acids can be used, and it is not necessary that the metal of the mercaptide and the metal of the salt be the same.

As an example of the efficacy of this novel ingredient, I cite below tests wherein an extreme pressure lubricant compounded with this novel ingredient was directly compared with a mineral lubricating oil (column 2) and with this oil containing stannic chloride (column 3). Oils of the type referred to herein may be tested upon the Almen pin test machine, described by Moughay and Almen, (Proc. A. P. I. 1931, page 77), wherein a pin is rotated in bearings so designed that increasing pressures may be applied to the lubricated surface. This machine is widely used in such comparative evaluations. In the following tabulation of results from the Almen pin test machine, the first column is the pressure in pounds per square inch applied to the lubricated contact surfaces. Columns 2, 3, 4 and 5 show the torque transmitted through the pin of the test machine, and show the pressure at which lubrication failed, resulting in seizure of the surfaces of the bearing and pin.

Table

| (1)                    | (2)          | (3)                       | (4)                       | (5)                       |
|------------------------|--------------|---------------------------|---------------------------|---------------------------|
| Pressure               | Oil<br>alone | Torque                    | Transmitted               | Foot-pounds               |
| Pounds per<br>sq. inch |              | Oil plus<br>0.1% $SnCl_4$ | Oil plus 0.1%<br>new base | Oil plus 2.0%<br>new base |
| 1000                   |              |                           |                           |                           |
| 2000                   | 0.5          | 0.5                       |                           | 0.5                       |
| 3000                   | Seized.      | 0.9                       | 0.8                       | 0.8                       |
| 5000                   |              | 1.5                       | 1.5                       | 1.4                       |
| 7000                   |              | 2.0                       | 1.8                       | 1.7                       |
| 8000                   |              | Seized.                   | 2.0                       | 1.8                       |
| 10000                  |              |                           | 2.1                       | 2.3                       |
| 15000                  |              |                           | 2.5                       | 1.9                       |
| 20000                  |              |                           | 3.0                       | 1.9                       |
| 24000                  |              |                           | 6.2                       | 4.1                       |
| 25000                  |              |                           | 6.3                       | Seized.                   |

In the tabulation given above, the oil used in column 2 was a cylinder stock having a viscosity of about 165 seconds Saybolt at 210° F. This oil is

an oil of the type normally used in the compounding of extreme pressure lubricants, and in the absence of special characterizing ingredients, may be used for such services, altho it is quite ineffective. The oil whose tests are reported in column 3, consists of the same oil as in column 2, containing 1% by weight of stannic chloride, which has a moderate capability alone as an E. P. ingredient, and this amount of stannic chloride is comparable with the amount of stannic chloride in an E. P. lubricant compounded with 1% of the novel base herein described. It will be observed that the oil of column 3 failed at a pressure of 8,000 pounds per square inch. Columns 4 and 5 show the tests of an E. P. lubricant composed of the oil of column 2 and containing 1% and 2% respectively of the novel characterizing ingredient herein described. It will be observed that the oils of columns 4 and 5 lubricated without seizure to loads far in excess of those at which failure was had with the hydrocarbon oil alone or with the hydrocarbon oil and an amount of stannic chloride corresponding to that present in the oil of column 4. The specific characterizing ingredient employed in the oil of column 4 was prepared by incorporating stannic chloride with

(iso-amyl)- $SCH_2COOH$ 

made from a pure mercaptide; the base used in compounding the oil of column 5 differed in that the original mercaptan-containing acid was prepared by use of a mixture of mercaptans boiling in the range of 100 to 135° C. Whether the product is made from pure or mixed mercaptides is immaterial to the effectiveness of the finished product, and whether the finished product contains 1% or 2% of the ingredient likewise makes little difference.

In the claims, the term "extreme pressure lubricating composition" means either (and includes all) the finished lubricant as actually used, the characterizing extreme pressure ingredient itself, or any intermediate extreme pressure lubricant base, admixture or dilution containing the active ingredient. The term "mercaptan-substituted fatty acid", as used in the claims, means the intermediate reaction product derived from the reaction between a mercaptide or mercaptides and a fatty acid or fatty acids, or metal salts thereof, within the scope of the detailed definitions given herein, said compound being of the general formula  $RS(CH_2)_xCOOH$ . The term "mercaptide" as used in the claims means any mercaptide or mixture of mercaptides; similarly the terms "fatty acid" and "metal salt" include both single and mixed fatty acids and salts.

## I claim:

1. An extreme pressure lubricating composition comprising hydrocarbon lubricating oil and a minor proportion of the reaction product of mercaptan-substituted fatty acid and stannic chloride.

2. A lubricant consisting mainly of relatively viscous hydrocarbon lubricating oil and a small amount of a reaction product of mercaptan-substituted fatty acid and stannic chloride sufficient at least to more than double the load carrying capacity of said lubricating oil as determined by the Almen pin test, substantially as described.

3. A lubricant consisting mainly of relatively viscous hydrocarbon lubricating oil and the reaction product of mercaptan-substituted fatty acid and stannic chloride sufficient greatly to increase the load carrying capacity of said lubricating oil but not in excess of 5% of said reaction

- product calculated upon the weight of the hydro-carbon oil present in the finished lubricant.
4. An extreme pressure lubricating composition comprising hydrocarbon lubricating oil and a minor proportion of the reaction product of mercaptan-substituted fatty acid selected from the group consisting of butyric acid to caprylic acid, inclusive.
5. An extreme pressure lubricating composition comprising a relatively viscous hydrocarbon lubricating oil and a minor proportion, sufficient to increase the load-bearing capacity, of a product secured by reacting a mercaptide and an alkali metal salt of a halogen substituted fatty acid to obtain a reaction product of the nature of a salt of a mercapto-acid, acidifying this salt to recover therefrom the said mercaptan-substituted fatty acid, and then reacting this acid with stannic chloride to obtain an active extreme pressure lubricating ingredient.
6. An extreme pressure lubricating composition comprising a major proportion of a hydrocarbon lubricating oil and a minor proportion, sufficient to increase the load-bearing capacity of a product prepared by reacting a mercaptide with at least one compound selected from the group consisting of chlor-substituted fatty acids and alkali metal salts thereof, acidulating the first reaction product to recover a mercaptan-substituted fatty acid, and reacting this acid with stannic chloride to obtain an active extreme pressure ingredient.
7. An extreme pressure lubricating composition comprising a major proportion of a viscous hydrocarbon oil and a minor proportion, sufficient to increase the load-bearing capacity of the mixture, of a product prepared by reacting a mercaptide with at least one compound selected from the group consisting of chlor-substituted fatty acids from butyric to caprylic, inclusive, and alkali metal salts thereof, acidulating the first reaction product to obtain a mercaptan-substituted fatty acid, and reacting this acid with stannic chloride to obtain the desired characterizing ingredient.

WILLIAM L. EVERSON.